# EUROPEAN PATENT APPLICATION

(11) **EP 0 518 840 A1**
(43) Date of publication of application: **16.12.1992**
(21) Application number: 92850139.4
(22) Date of filing: 10.06.1992
(51) Int. Cl.: C22C 29/04, C22C 1/05

(54) **Method of making sintered carbonitride alloys**

(30) Priority: 12.06.1991 SE 9101799
(71) Applicant: SANDVIK AKTIEBOLAG, S-811 81 Sandviken 1 (SE)
(72) Inventor: Weinl, Gerold, S-125 51 Älvsjö (SE); Östlund, Ake, S-183 46 Täby (SE); Jutterström, Ulf, S-112 53 Stockholm (SE)
(74) Representative: Östlund, Alf Olof Anders

(57) **Abstract**

According to the present invention there is now provided a method of manufacturing a sintered body of titanium based carbonitride alloy comprising hard constituents in 525 % binder phase where the hard constituents contain, in addition to Ti, one or more of the metals Zr, Hf, V, Nb, Ta, Cr, Mo or W and the binder phase is based on cobalt and/or nickel with powder metallurgical methods, i.e., milling, pressing and sintering. If the powder to be compacted has a mean agglomerate size of 40-80 µm and a span of <1.5 less porosity and lower compaction pressure is obtained.

## Description

The present invention relates to a method of manufacturing sintered titanium based carbonitride alloys with powder metallurgical methods. By using a powder with a certain agglomerate size and distribution it has turned out that lower compaction pressure as well as lower porosity can be obtained.

Sintered titanium based carbonitride alloys, so-called cermets, are today well established as insert material in the metal cutting industry and are especially used for finishing. They contain mainly carbonitride hard constituents embedded in a binder phase. The hard constituent grains generally have a complex structure with a core surrounded by a rim of other composition. Their grain size is usually <2 µm.

In addition to Ti, other metals of the groups IVa, Va and VIa, i.e., Zr, Hf, V, Nb, Ta, Cr, Mo and/or W, are normally found in the carbonitride hard constituents but may also be present as carbide and/or nitride hard constituents. The binder phase generally contains cobalt as well as nickel. The amount of binder phase is generally 5 - 25 % by weight.

Sintered carbonitride alloys are as conventional cemented carbide manufactured by powder metallurgical methods, namely, milling, pressing and sintering. The milling is generally performed in an inorganic milling liquid and normally together with a pressing agent. The object of the pressing agent is to act lubricating during the subsequent tool pressing. The pressing agent, however, also has another object, namely, to protect the fresh surfaces resulting from the milling against oxygen pick up. After the milling the milling liquid is removed usually by spray drying. By a proper choice of conditions during the spray drying spherical agglomerates are obtained with desired size and size distribution. These agglomerates are more or less completely covered by the pressing agent. The larger the size of the agglomerates is, the more favourable ratio surface/volume such agglomerates have. It can, thus, be expected that materials sensitive to oxygen shall have as large agglomerate size as possible in order to minimize this oxygen pick up.

The size and distribution of the agglomerates can be determined by sieving or in any other way and can be characterized by the mean agglomerate size, C, and the span defined by (A-B)/C, where A = the agglomerate size below which 90% of all agglomerates are found and B = the agglomerate size below which 10% of all agglomerates are found.

For conventional cemented carbide a mean agglomerate size of 100-150 µm with a span <2 has been found suitable. It has now surprisingly turned out that for titanium based carbonitride alloys the mean agglomerate size shall be 40-80 µm, preferably 40-60 µm and the span <1.5, preferably <1.2. In this way lower compaction pressure and less porosity is obtained than if the usual mean agglomerate size for conventional cemented carbide is used.

High compaction pressure is linked to an increased risk for the generation of cracks as well as uneven density distribution in connection with the compaction. The presence of cracks and uneven density distribution can lead to problems with crack generation as well as deviations in dimension in the sintered carbonitride alloy. The presence of pores also can result in deviations in dimensions and influence on the mechanical properties of the finished alloy.

The type of porosity which easily arises in carbonitride alloys manufactured using agglomerates with a mean agglomerate size corresponding to that for normal cemented carbide, i.e., 100-150 µm is often so called agglomerate porosity, i.e., the original agglomerates are visible and material has not filled the voids between them. Such porosity can be very disastrous since these pores are relatively large, on one hand, and can be angular and have a strong notch effect, on the other. Carbonitride alloys as such are from a general point of view more brittle than cemented carbide and have more difficulty to stop possible cracks. They are, thus, more notch sensitive than cemented carbide.

The present invention, thus, relates to a way of manufacturing carbonitride alloys using a powder with a mean agglomerate size which is considerably smaller that the size which has turned out to be suitable for conventional cemented carbide. In spite of the general relations between oxygen pick up and agglomerate size the decrease of mean agglomerate size leads to improved properties such as lower compaction pressure and less porosity. As a result a densely sintered product with less deviations in dimensions is obtained.

### Example

Titanium based carbonitride alloys with the following composition in weight-% 15 W, 39.2 Ti, 5.9 Ta, 8.8 Mo, 11.5 Co, 7.7 Ni, 9.3 C, 2.6 N were manufactured with an agglomerate size of 125 µm and span 1.8, A, and with an agglomerate size of 55 µm and span 1.1, B, (according to the invention). During pressing the compaction pressure was measured and after sintering the porosity was evaluated. Sintering took place in vacuum at 1430°C for 90 min.

## Claims

1. Method of manufacturing a sintered body of titanium based carbonitride alloy comprising hard constituents in 5-25 % binder phase where the hard constituents contain, in addition to Ti, one or more of the metals Zr, Hf, V, Nb, Ta, Cr, Mo or W and the binder phase is based on cobalt and/or nickel by powder metallurgical methods, i.e., milling, pressing and sintering **characterised** in that the powder to be compacted is agglomerated with a mean agglomerate size of 40-80 µm and a span of <1.5.
